

# UNITED STATES PATENT OFFICE.

MARCO BIROLI, OF PAVIA, ITALY.

## PROCESS OF PRODUCING GLOSSY THREADS FROM VISCOSE.

1,226,178.

Specification of Letters Patent. Patented May 15, 1917.

No Drawing.

Application filed November 18, 1916. Serial No. 132,108.

*To all whom it may concern:*

Be it known that I, MARCO BIROLI, a subject of the King of Italy, residing at 3 Piazza Carmine, Pavia, Italy, have invented 5 certain new and useful Improvements in Processes of Producing Glossy Threads from Viscose, of which the following is a specification.

This invention relates to a process for producing glossy threads from viscose.

Processes are already known for directly obtaining cellulose threads, which are, however, not xanthogenate threads, by means of a bath of bisulfate and sulfuric acid, such 15 a process being disclosed in Müller, No. 836,452, of November 20, 1906.

According to the present invention, sodium bisulfate alone is used. To produce such a thread, it is necessary to adopt such a degree 20 of concentration of the solution, such a temperature and such a mechanical arrangement that, after the issue of the viscose from the drawing plate, a xanthogenate thread is formed in the coagulation bath. This 25 xanthogenate thread, in a further phase, is transformed into a cellulose thread by being passed into a fixation bath consisting of a suitable diluted acid. The degree of concentration of the acid salt solution must be so 30 adjusted that only a moderate degree of decomposition is obtained. It has been found that a 27% solution of sodium bisulfate, without the addition of sulfuric acid and under determined temperature conditions, 35 average 50° C., for instance, may be successfully used.

To the combinations which are not capable

of decomposing the xanthogenate for themselves, but require further treatment of the thread by a fixation liquid, belong the solutions of salts and organic acids.

It has been found that the following solutions give the best results:—

First. Nearly saturated sodium chlorid solution containing 10% of industrial acetic acid.

Second. Magnesium sulfate solution containing 10% of acetic or formic acid.

The artificial silk threads manufactured according to the present process possess 50 high technical value, as they are superior to all other viscose threads for their bright gloss, softness of touch and strength.

What I claim is:—

1. The process of producing glossy threads from viscose which consists in passing the viscose threads into a bath of sodium bisulfate with the formation of xanthogenate, and then passing the resulting threads into a solution containing an organic acid radical.

2. The process of producing glossy threads from viscose which consists in passing the threads into a bath of sodium bisulfate with the formation of xanthogenate, and then passing the resulting threads into a bath of suitable salts and organic acids to cause the decomposition or fixation of the xanthogenate threads.

In testimony whereof I affix my signature in presence of two witnesses.

MARCO BIROLI.

Witnesses:

LUIS F. HEMÁUDER,  
IVAN LAVRETSKY.